

## UNITED STATES PATENT OFFICE

2,091,143

DYEING BY MEANS OF SULPHURIC ESTERS  
OF INDAANTHRONES

David Alexander Whyte Fairweather, Falkirk, and John Thomas, deceased, late of Polmont, Scotland, by Olive Morgan Thomas, Wilmslow, and Barclays Bank Limited, Manchester, England, executors, assignors to Imperial Chemical Industries Limited, a corporation of Great Britain

No Drawing. Original application April 16, 1931, Serial No. 530,724. Divided and this application June 10, 1935, Serial No. 25,938. In Great Britain April 16, 1930

10 Claims. (Cl. 8—5)

This invention relates to improvements in dyeing by means of sulphuric esters of indanthrones, and it comprises methods of dyeing cotton, wool and other fibers and the like wherein the material to be dyed is impregnated with tri- and di-esters of an indanthrone compound, in the form of the azine and the color is then developed by removing the sulphuric ester groups by hydrolysis, advantageously by acid hydrolysis using dilute solutions of mineral acids, the azine structure being simultaneously converted into a dihydroazine nucleus during the formation of the final shade or color. This invention is particularly directed to dyeing processes wherein the said material is impregnated with an azine di-ester, such as anthraquinoneanthrahydroquinoneazine disulphuric ester alkali metal salt, and the color developed by means of dilute mineral acid, without the use of oxidizing agents.

20 This application is a division of our copending application Ser. No. 530,724, filed April 16, 1931 (U. S. Patent 2,019,530, November 5, 1935).

According to the present invention the di-sulphuric leuco ester of indanthrone in the azine form may be applied to the cloth and developed by a more simple procedure than heretofore required for the known sulphuric acid esters of indanthrone. In preparing the dyebath we obtain higher concentrations of potential coloring matter, calculated as indanthrone. We obtain increased actual solubility by the presence of sulphuric ester groups and obtain a higher percentage of potential coloring matter due to the fact that the ester contains fewer of these ester groups. In developing the color on the material to be dyed, a relatively smaller amount of salts of sulphuric acid are formed.

The greatest advantage of our processes is that development of color can be obtained without the use of oxidizing agents or with a minimum of such agents when their use becomes necessary. By using the sulphuric esters in the form of the azine, at least half of the necessary oxidation is obtained by internal rearrangement of the structure of the dye. This rearrangement is explained more fully post. This remarkable property of self-oxidation facilitates maintaining the amount of oxidizing agent, below that which produces the said greening of the final shade, in those cases

in which the oxidizing agent cannot be entirely eliminated.

With the azine di-esters which are completely self-oxidizing, removal of the ester groups effects an automatic formation of the exact final coloring matter desired; the hydroxyl groups so produced, the presence of which is indicative of undeveloped coloring matter, give rise to internal rearrangements by which azine structures are converted into the desired dihydroazine nucleus. The oxidizing action being within the compound itself, no arbitrary fixing of the oxidation is required. Greening of the final shade and undeveloped coloring matter are, so to speak, automatically avoided. The major precaution required is to provide sufficient time and acid to effect complete hydrolysis and leave substantially no sulphuric ester on the material to be dyed. If a small amount of sulphuric ester does remain, it can easily be removed by suitable washing because of its comparatively greater solubility.

The tri- and di-ester useful in our dyeing methods may be prepared by various processes.

In our copending application Serial No. 25 530,724, of which the present application is in part a division and in part a continuation, there is described the preparation of a large number of such sulphuric esters. That application is directed to the methods of so making these esters 30 and to the trisulphuric esters formed as an intermediate product. The present application is directed to the dyeing procedures using those esters.

While we find it advantageous to use the esters 35 in the azine form, dihydroazines may be used. However, they should be converted into the azine form before the final development of color is effected.

The di-esters most advantageous in the present processes are the di-esters of an anthraquinoneanthrahydroquinoneazine. 3:3'-dichloroanthraquinoneanthrahydroquinoneazine disulphuric ester and anthraquinoneanthrahydroquinoneazine disulphuric ester are typical. Such 45 di-esters, as a class, are self-oxidizing; these azine esters being converted into a corresponding dihydroazine dianthraquinone by treatment with dilute solutions of mineral acid.

In our dyeing processes, using such azine di- 50

esters, the dyestuff may be applied to the material in various ways. Padding methods, printing procedures, etc., may be employed.

Suitable dyebaths may be prepared by dissolving the azine di-ester in water or aqueous solutions. Ordinarily the di-ester is employed in the salt form, usually as the alkali metal salt, (sodium salt). Cloth, yarn and the like may be impregnated by means of these dyebaths or solutions in the usual manner. Then the impregnated material, with or without drying, is developed by treatment with dilute acid. Dilute solutions of mineral acids, such as sulphuric and hydrochloric acids may be used. No added oxidizing agent is required, the color being automatically developed by this acid treatment.

Printing pastes may be prepared with the azine di-ester and cloth printed in the usual manner. For instance, printing pastes may be prepared by mixing the azine di-ester with glycerine and gum tragacanth solution in suitable proportions. The printed cloth may likewise be developed with dilute solutions of mineral acids; no added oxidizing agent being necessary.

25 The following examples illustrate dyeing processes using the azine di-esters:

#### Example 1

30 This example illustrates dyeing with 3:3'-dichloro - anthraquinoneanthrahydroquinoneazine disulphuric ester (prepared, for instance, by the process of Example 16 of U. S. Patent 2,019,530).

Cotton cloth is padded at about 40° C. with 35 concentrated solution of the said ester and then, with or without drying, passed through a 0.5 per cent solution of hydrochloric acid.

A deep bright blue shade immediately develops apparently corresponding to 3:3'-dichloro-40 indanthrone.

#### Example 2

This example illustrates a printing process using 3:3'- dichloro-anthraquinoneanthrahydro-45 quinoneazine disulphuric ester.

The printing paste is made up as follows:—

|                           | Parts |
|---------------------------|-------|
| Diester                   | 20    |
| Glycerine                 | 5     |
| 50 Gum tragacanth (5:100) | 75    |
|                           | 100   |

The paste is printed on cotton or on woolen cloth, dried, aged for ten minutes, developed in 55 1% hydrochloric acid at 60° C., and rinsed in soap.

#### Example 3

60 This example illustrates a dyeing method using anthraquinoneanthrahydroquinoneazine disulphuric ester.

One part of the anthraquinoneanthrahydroquinoneazine disulphuric ester is dissolved in 100 65 parts of water, the temperature is raised to about 60° C. and 10 parts of cotton yarn entered and kept at about 60° C. for half an hour, salt being added to assist exhaustion. The yarn is dyed in orange-red shades. The yarn is removed and immersed in a bath containing 1 per cent hydrochloric acid at 50° or 60° C. for a few minutes, the said red-orange shades being converted by this acid treatment to blue.

70 75 The following examples illustrate dyeing proc-

esses using an anthraquinoneanthrahydroquinoneazine disulphuric ester containing nuclear hydroxyl groups. Such compounds containing these nuclear hydroxyls may be prepared by boiling an alkali metal salt of dianthrahydroquinone tetrasulphuric ester with caustic soda solution until two sulphuric ester groups are removed by hydrolysis. (See Example 7 of U. S. Patent 2,019,530).

#### Example 4

10

This example illustrates dyeing processes using an anthraquinoneanthrahydroquinoneazine disulphuric ester containing nuclear hydroxyl groups obtainable as described ante.

Two parts of a 10 per cent paste of the said azine di-ester are dissolved in 200 parts of water and 10 parts of cotton cloth is entered at 60° C. and worked at that temperature for 30 minutes. 10 parts of sodium chloride are then added to the dyebath and the dyeing continued for a further 30 minutes.

The cotton is thus colored a reddish brown which is changed to a bright blue by immersion in a 1 per cent solution of sulphuric acid at 15° C. 25 The blue shade is not so red as the shade of dianthraquinone dihydroazine and the body may be a dianthraquinone dihydroazine derivative. This appears to represent a simpler method of obtaining a dyeing of a dianthraquinone dihydroazine derivative than any previously described whether by the vat or soluble ester methods.

#### Example 5

35

This example illustrates another method of dyeing with the dyestuff used in Example 4.

10 parts of woolen cloth well wetted out are entered into the dyebath as used in Example 4, and the temperature raised to 70° to 75° C. 40 Exhaustion is effected by the cautious addition of dilute acetic acid.

The dyeing which already is somewhat blue in color towards the end of the process, is immersed for 5 minutes in a 1 per cent solution of sulphuric acid at 15° C., when a bright blue shade is developed.

In the foregoing illustrative examples of dyeing methods, it is to be noted that the development of color is effected by treatment with dilute mineral acids; no oxidizing agent being required. This is a feature of such processes and an advantage of our new azine di-esters. These new azine di-esters are, so to speak, self-oxidizing, that is, when the two ester groups are removed by hydrolysis with the dilute mineral acid, the hydroxyl groups so formed are oxidized by internal rearrangement involving conversion of the azine ring into a dihydroazine structure.

The di-esters of an anthraquinoneanthrahydroquinoneazine may be prepared from the tetrasulphuric esters of a dianthrahydroquinoneazine, by the two-step method described in our copending application Serial No. 530,724, wherein one sulphuric ester group is first removed from the tetra-ester by a restricted acid hydrolysis or by hydrolysis in an aqueous medium in the presence of a reducing agent, and then a second sulphuric ester group removed by hydrolysis in an aqueous medium in the presence of an oxidizing agent. 60 The details of such processes, as applied to the tetrasulphuric ester of 3:3'-dichloro-dianthrahydroquinoneazine and of dianthrahydroquinoneazine are set forth in the aforesaid copending application.

75

These new azine di-esters of an anthraquinone-anthrahydroquinoneazine contain as the characteristic nucleus the following nucleus (represented in the form of the sodium salt):

5



10

15

20

30

35

40

55

60

65

Such azine di-esters, per se, are new. The anthraquinoneanthrahydroquinoneazine disulphuric ester is believed to have, in the form of the sodium salt the following formula:

It is a bright red body having good solubility in water. Its solution in water is not colored violet by the addition of caustic alkali. On reduction with sulphide and hydrosulphite and alkali, the color of the solution changes to blue green. On treatment with dilute mineral acid the vat dyestuff indanthrone is precipitated.

The 3:3'-dichloro-anthraquinoneanthrahydroquinoneazine disulphuric ester is believed to have, in the form of the sodium salt, the following formula:



It is likewise a red soluble ester. Its properties are similar to those of anthraquinoneanthrahydroquinoneazine disulphuric ester; dichloro-indanthrone being precipitated on treatment with dilute mineral acid.

The development of an indanthrone coloring matter from the azine di-ester upon treatment with dilute mineral acid, is shown diagrammatically as follows; anthraquinoneanthrahydroqui-

noneazine disulphuric ester being used for purposes of illustration:



From the foregoing showing it is clear that the dilute mineral acid effects removal of the two sulphuric ester groups forming two hydroxyl groups. Then migration of the hydrogen of those hydroxyl groups to the azine ring, effects conversion of the azine into dihydroazine with simultaneous oxidation of the said hydroxyl groups. This is what is here called "self-oxidation"; oxidation by internal rearrangement. Thus the development of the desired coloring matter is automatically obtained; the desired dihydroazine form and oxidation of hydroxyls being produced upon hydrolysis.

This internal rearrangement is characteristic of these azine di-esters as a class.

While an essential feature of our new dyeing processes is this self-oxidation, and the use of such azine di-esters, it is not mandatory to use the azine di-ester as a starting material or dyestuff. Our processes may be practiced using other esters, as the starting material or dyestuff, and forming the azine di-ester during the processing. For instance, a tri-sulphuric ester may be applied to the material to be dyed and then the azine di-ester produced in situ, before development of the final color, by a suitable treatment. The azine di-ester may be formed in situ, to advantage, by subjecting the cloth impregnated with a di-ester to treatment with an alkaline solution of an

5

10

15

20

25

30

35

40

45

50

55

60

65

70

75

oxidizing agent; this treatment being controlled to remove one sulphuric ester group and form an azine compound. The so treated cloth may be further treated to eliminate any excess of 5 oxidizing agent before final development of color with acid. Sodium sulphite may be used to destroy excess of hypochlorite when that substance is used as the oxidizing agent.

Again, the dyebath may be prepared by dissolving 10 a tri-ester in an alkaline aqueous solution or water and then forming the azine di-ester in situ before cloth or yarn is entered into the bath; the azine di-ester being advantageously formed in situ by adding a suitable amount of 15 oxidizing agent or alkaline solution thereof to the dyebath. After the reaction is complete, any excess of oxidizing agent should be removed or destroyed before application of the ester to the cloth. Using a hypochlorite as the oxidizing 20 agent, any excess may be reacted with the required amount of a sulphite, such as sodium sulphite to eliminate it. Other oxidizing agents such as alkali metal persulphates, bleach liquors, etc., may be used.

25 In these modifications of the generic processes, the development of the final color is by means of dilute mineral acid without the presence of added oxidizing agents.

30 The following examples illustrate the application of the modifications mentioned ante, to dyeing processes:

#### Example 6

This example illustrates a dyeing method 35 wherein an azine tri-ester is applied to the cloth and the azine di-ester is produced in situ upon the cloth prior to development to the final color.

0.2 part of dianthrhydroquinoneazine trisulphuric ester are dissolved in 200 parts of water 40 together with 10 parts of sodium chloride and 10 parts of cotton cloth entered at 50° C. and worked for 30 minutes. The dyeing which has a reddish orange shade is squeezed and immersed in a bath containing 1 per cent of sodium hypochlorite, 2 per cent of caustic soda and 10 per cent of sodium chloride for one minute at 50° C. The shade 45 changes toward the red, and the cloth is now squeezed and run through a 2 per cent bath of sodium sulphite being finally developed in a 1 per cent sulphuric acid bath at 60° C. when a blue shade is produced.

In this example treatment of the cloth impregnated with the tri-ester, with the solution of sodium hypochlorite, forms the anthraquinone-anthrhydroquinoneazine disulphuric ester in 55 situ on the cloth. The treatment with sodium sulphite is to eliminate any excess of the oxidizing agent. The treatment with dilute sulphuric acid, as specified, forms the final coloring matter by hydrolysis and internal rearrangement of the 60 dyestuff.

In Example 6, other azine tri-esters might be used, for instance, 3:3'-dichloro-dianthrhydroquinoneazine trisulphuric ester. Likewise dilute solutions of other mineral acids, for instance, 65 hydrochloric acid, might be used to develop the final color. Further, the other suitable oxidizing agents might be used in lieu of the sodium hypochlorite to form the azine di-ester in situ.

This method of developing the azine di-ester 70 in situ on the cloth from a tetra-ester, is not limited to using azine tri-esters. It may be also practiced with other tri-esters, for instance, anthranoanthrhydroquinone dihydroazine trisulphuric ester. The following example illustrates 75 the use of such an anthranol compound.

#### Example 7

In this example the tri-ester of anthranol-anthrhydroquinone dihydroazine is used. This tri-ester is somewhat different from the tri-ester used in Example 6 and it may be represented in the form of sodium salt by the following formula:



0.2 part of the anthranolanthrhydroquinone dihydroazine trisulphuric ester, are dissolved in 200 parts of water together with 10 parts of sodium chloride, and 10 parts of cotton cloth 25 entered at 50° C. and worked for 30 minutes.

The deep orange-red dyeing is squeezed and immersed in a bath containing 1 per cent of sodium hypochlorite, 2 per cent of caustic soda and 10 per cent of sodium chloride for 1 minute at 50° C. The shade changes towards brown, and the cloth is now squeezed and run through a 2 per cent bath of sodium sulphite, being finally developed in a 1 per cent sulphuric acid bath at 60° C. when a blue shade is produced.

In this example, the treatment with alkaline hypochlorite solution not only converts the dihydroazine into an azine compound, but also oxidizes the anthranol structure into an anthraquinone nucleus simultaneous with the removal of one sulphuric ester group, thus producing anthraquinoneanthrhydroquinoneazine disulphuric ester in situ. This procedure may be used with any of the tri-sulphuric esters obtainable from the tetrasulphuric ester by a stronger reduction treatment than is necessary to form the tri-esters of dianthrhydroquinoneazine.

The following example illustrates the formation of azine disulphuric ester from a trisulphuric ester in situ in the dyebath before the dyestuff is applied to the material to be dyed.

#### Example 8

200 parts of a 10 per cent paste (calculated as indanthrone) of dianthrhydroquinoneazine tri-sulphuric ester, together with 400 parts of water and 50 parts of 20 per cent caustic solution are warmed to 50° C. When the tetrasulphuric ester has dissolved, 12.5 parts of potassium persulphate are gradually added. When the addition is complete the temperature is raised to 70° C. for half an hour. If necessary, sodium sulphite may then be added to eliminate any excess persulphate if present. The liquor so obtained may be filtered if desired.

This solution is an advantageous dyebath for use in our dyeing processes. It may be used according to the dyeing processes of Examples 1, 3 and 4; the red solution obtained in this example, being used in lieu of the solutions of anthraquinoneanthrhydroquinoneazine disulphuric ester disclosed in the said examples. The procedures to be followed are substantially the same; the final color being developed by dilute solution of mineral acid.

Of course other azine di-esters might be formed in situ in the dyebath prior to applying the dyestuff to the cloth, yarn, etc., from other tri-esters.

Although in our processes it is advantageous to 5 form the azine di-ester before the impregnated material is treated with mineral acid to develop the final color, our processes may be practiced using the tri-sulphuric esters and simultaneously forming the azine disulphuric ester and developing 10 the final color with mineral acid. In this modification of our processes, the tri-ester is applied to the material to be dyed and then the impregnated material is treated in a developing bath comprising a dilute solution of acid containing 15 an oxidizing agent dissolved therein. Such developing baths may be prepared by dissolving copper sulphate and like oxidizing agents in dilute solutions of mineral acid, such as sulphuric and hydrochloric acids. About 1 per cent mineral 20 acid and approximately 2 per cent copper sulphate give baths of suitable concentration for ordinary use. The amount of oxidizing agent used should be merely sufficient to oxidize one pair of hydroxyl groups (formed by acid hydrolysis) 25 to the desired quinone "oxygens"; the other pair of hydroxyls (so formed) being oxidized by internal rearrangement with the formation of the dihydroazine compound. In this way over oxidation can be easily avoided.

30 The following examples illustrate such processes using the azine trisulphuric esters.

#### Example 9

35 In this example cotton yarn in the form of hanks are dyed with indanthrone coloring matter derived from dianthrahydroquinoneazine tetrasulphuric ester.

20.5 parts of a solution of dianthrahydroquinoneazine trisulphuric ester, containing the equivalent of 1 per cent indanthrone, are made up to 410 parts with water and heated to 60° C. 40 20.5 parts of cotton hanks are wetted out and immersed in the bath so prepared, and after working for half hour 30.5 parts of common salt are added. After a final half hour's working the hanks are lifted, wrung and immersed for about 5 minutes in a solution of 1 per cent copper sulphate crystals, 1 per cent of concentrated hydrochloric acid at 85-90° C. This causes the reddish 45 color to pass through purple to bright blue. The hanks are removed, washed, soaped, washed and finished. The material, if desired, may be padded in a normal way in a somewhat stronger bath of 50 any strength, and after squeezing and drying is 55 steamed and developed.

#### Example 10

60 This example illustrates dyeing woolen cloth

using dianthrahydroquinoneazine trisulphuric ester as the dyestuff.

One part of dianthrahydroquinoneazine tri-ester is dissolved in 200 parts of water at 50° C. and the temperature raised to 70° C. 5 parts of 5 woolen cloth, which has been scoured for 5 minutes in 1 per cent ammonia solution at 95° C., are then entered. The cloth is worked for 15 minutes during which time the temperature is raised to the boil and dyeing is continued for 10 minutes at this temperature. 5 parts of common salt are added at intervals during a further 20 minutes, the cloth being worked during this period. The material is then raised and squeezed before developing in the following solution for 15 three minutes at 100° C.:

|                   | Per cent |
|-------------------|----------|
| Copper sulphate   | 2        |
| Hydrochloric acid | 1        |

20 The dyeing is washed in water, soaped for 5 minutes at 60° C. in 1 per cent soap solution, washed and dried.

#### Example 11

25 This is an example of a printing method using dianthrahydroquinoneazine trisulphuric ester.

30 This printing paste is made up as follows:

|                                              | Parts |
|----------------------------------------------|-------|
| Dianthrahydroquinoneazine trisulphuric ester | 20    |
| Glycerine                                    | 5     |
| Gum tragacanth (5:100)                       | 75    |
|                                              | 100   |

40 The paste is printed on cotton or on woolen cloth, dried, aged for 10 minutes and developed in 1 per cent hydrochloric acid and 2 per cent copper sulphate solution at 90° C., rinsed and soaped.

45 The tri-esters used in the foregoing examples may be prepared from the tetrasulphuric esters by treating said tetra-esters with reducing agents in an aqueous medium. Generically such processes comprise the controlled removal of a single sulphuric ester group, the treatment being stopped at that point. Such processes are described in detail in our copending application Serial No. 530,724.

50 Preferably the trisulphuric esters are prepared 55 in the form of the azine compound for use in these dyeing processes. Such tri-esters may be represented using dianthrahydroquinoneazine trisulphuric ester as an illustration, by the following isomeric formulae:



The conversion of these trisulphuric esters may be diagrammatically represented as follows, using the same tri-ester as an illustration:

5

10

15

20

25

30

35

40

45

50

55

60



In all our processes, we believe that two or 65 more of the above changes or conversions are involved. In our processes wherein a trisulphuric ester is applied to the cloth or other materials to be dyed, and the final color developed in a bath containing both acid and an oxidizing agent, 70 we believe that all of these changes occur in

rapid succession; the rapidity of action being so great that these complex changes appear to be a single change. However, we believe as even in that case, there is the conversion of anthraquinoneanthrahydroquinoneazine into dianthrhydroquinoneazine. That such is a fact, is evidenced by the development of the final color with an amount of oxidizing agent only half of that required to theoretically convert the four hydroxyls of dianthrhydroquinoneazine into quinone oxygens. Thus we believe that in all of our processes at least half of the required oxidation is a self-oxidation involving internal rearrangement within the dyestuffs; a dihydroazine being the final product.

In the foregoing examples, the parts given are parts by weight. Those examples, merely illustrate our invention and in no way are to be considered limiting the scope of this invention.

While we have specifically mentioned the alkali metal salts of these sulphuric esters, our processes are not limited to such salts. Any suitable salt of these esters may be used. Generically our invention is applicable to these tri- and di-sulphuric esters as a class.

What we claim is:—

1. In the process for dyeing fibers with indanthrone dyestuffs, the improvement which comprises impregnating the fiber with an aqueous solution of a disulphuric leuco ester of indanthrone in the azine form and precipitating the color in the fiber by treating the same with a dilute solution of an acid, in the absence of an oxidizing agent.

2. The process of claim 1 wherein the disulphuric acid ester with which the fiber is impregnated is the leuco disulphuric ester of anthraquinoneanthrahydroquinoneazine.

3. The process of claim 1 wherein the said azine disulphuric ester is formed in situ on the material to be dyed.

4. As an improved process of dyeing with indanthrone dyes, the process which comprises applying to the fiber to be dyed an aqueous solution of a disulphuric ester of a leuco indanthrone in the azine form and subsequently contacting the fiber impregnated with said azine di-ester, with a dilute solution of mineral acid, in the absence of an oxidizing agent.

5. The improved process of claim 4 wherein a trisulphuric leuco ester of a reduced indanthrone is dissolved in an aqueous solution, an oxidizing agent is added to said solution, the said tri-ester is converted into an azine di-ester in the presence of said oxidizing agent, the excess oxidizing agent is eliminated, the solution of azine di-esters thus produced is applied to a textile material and the textile material impregnated with said azine di-ester is subsequently contacted with a dilute solution of mineral acid to develop the final color.

6. As an improved process of dyeing with indanthrone dyes, the process which comprises dissolving an anthraquinoneanthrahydroquinoneazine disulphuric leuco ester in an aqueous solution, impregnating the material to be dyed with said solution, and subsequently immersing the impregnated material in a dilute solution of a mineral acid, in the absence of an oxidizing agent.

7. The process of claim 6 wherein said mineral acid is hydrochloric acid.

8. The process of claim 6 wherein said mineral acid is sulphuric acid.
9. As an improved process of dyeing with indanthrone dyes, the process which comprises impregnating a textile material with an aqueous solution of a trisulphuric leuco ester of a reduced indanthrone, treating the impregnated textile material with an oxidizing agent to form an azine di-ester in situ, and subsequently developing the final color by contacting the so-treated textile material with a dilute solution of mineral acid.
10. The process of claim 9 wherein said oxidizing agent is an alkaline hypochlorite solution.

DAVID ALEXANDER WHYTE  
FAIRWEATHER.

5

OLIVE MORGAN THOMAS,  
BARCLAYS BANK, LTD.,  
*Manchester Trustee Dept.,*

By THOMAS ERIC SONE,

*Manager.*

10

*Executors of the Estate of John Thomas, Deceased.*